

Patented July 13, 1926.

1,592,294

# UNITED STATES PATENT OFFICE.

ALBERT L. CLAPP, OF DANVERS, MASSACHUSETTS.

## METHOD OF MAKING WATERPROOF PAPER OR FIBER BOARD.

No Drawing.

Application filed November 6, 1923. Serial No. 673,215.

This invention relates to waterproof paper or fiber board, such for example as is suitable for use as a wrapper or container for food products. 5 It also relates to the method of manufacture of this paper or fiber board by which the waterproofing material is incorporated in the paper stock so that the waterproof paper is completely formed on the paper machine, no subsequent saturation with the waterproofing material being necessary. By this method it is possible to form paper with a waterproof liner backed by other kinds of paper. This is of advantage, as for example, in the manufacture of paper pails and boxes, such as are commonly used for oysters, ice cream, etc., the waterproof liner being on the inside of the container where it contacts with the food and the outside of the container being of a nature to readily receive printing thereon, since printing can not be satisfactorily done on the waterproofed paper. The outside liner may also be made of cheap material such as news-paper, thus materially cheapening the material without in any way impairing its suitability for the purpose intended.

Heretofore it has been proposed to incorporate waterproofing material such as paraffin in the beater stock by forming an emulsion of the paraffin in a more or less saponified aqueous mixture. In practice, however, it has been found commercially impossible to run such a stock on a paper machine, as the emulsion forms a sticky mass which clogs the cylinder mold or Fourdrinier wire, and sticks to the blankets. The saponified mixture holds much water in combination and aside from the trouble from sticking it is a difficult matter to drive this off by the action of the drying rolls of the paper machine. The paraffin is also contaminated by a comparatively large amount of saponified salts and so fails to be wholly effective in waterproofing the paper.

A fine dispersion of paraffin or other waterproof material, however, may be made in an aqueous solution of a nature which permits the waterproofing material to be fixed as fine particles or granules to the fibers of a paper stock and without the production of any sticky substances which may stick to the blankets of the paper machine or clog the cylinder molds or Fourdrinier wire by the method described and claimed in

my application for patent entitled Dispersion product and method of making, Serial No. 673,216, filed Nov. 6, 1923.

A paraffin dispersion product may be prepared by melting together paraffin, rosin, and Montan or carnauba wax, suitable proportions being 900 parts of paraffin, 100 parts of rosin and 10 parts of Montan or carnauba wax, the Montan wax being somewhat preferable. This melted mixture is then poured into a solution of silicate of soda comprising 200 parts of silicate of soda and 1500 parts of water, the mass being thoroughly stirred and agitated while the mixture is being effected. While continuing the stirring the mixture is then cooled suddenly below the melting points of the waxes and rosin as by means of the addition of 2250 parts of cool or cold water, the stirring being continued until the wax and rosin appears as finely dispersed particles in the solution. While the paraffin in itself may be dispersed in the aqueous solution, yet the Montan or carnauba wax, being of greater penetrability and of lower surface tension than the paraffin, acts to permit a fine dispersion of the wax in the solution.

By the present method, therefore, the paraffin and Montan or carnauba waxes and the rosin are dispersed in finely divided or granular form in a silicate of soda solution, the mixture being non-sticky. This mixture has the physical characteristics of inert granular material in a sodium silicate solution. I do not herein claim per se the method of effecting a dispersion of the paraffin or other water-immiscible compound or composition.

The procedure in the production of the paper may be as follows: 5 to 45 parts of paraffin dispersion product, made according to a method heretofore described, are added to 55 to 80 parts of beaten sulphite pulp and thoroughly mixed therewith, 5 to 25 parts of alum or other precipitant may then be added and mixed in for a few minutes to form a flocculent precipitate with the silicate which acts to fix the dispersed material on the pulp. The sodium silicate acts as a coagulant to fix the dispersed particles over the fibers. The stock may then be run off on the paper machine and may be passed over heated calender rolls which causes the dispersed grains to flux together throughout the material. This stock is found to run as well or better on the paper machine than

though the paraffin were not present. No water is held mechanically combined so that the sheeted stock is readily dried by the usual drier rolls of the paper machine. By 5 heating the sheet so prepared above the melting point of the dispersed material in the fluxing operation, the particles coalesce and form an unbroken layer of waterproof and water repellent material entirely surrounding each fiber and filling the interstices between the fibers. The resultant product, therefore, is not only waterproof, but is water repellent comparable in this respect to paper which has been dipped in melted 10 paraffin.

So far as I am aware I am the first to produce a paper having these characteristics where the paraffin is incorporated in the pulp before it is sheeted on the paper machine. The product is quite different from a paper water-proofed by size such as rosin size. The rosin soap in rosin size is precipitated on the fibers in the form of a resinate which is incapable of being fluxed without 15 great heat so as to form a coating entirely encasing each fiber. By the method of this invention, however, the waxes, and nearly all of the rosin as free rosin is deposited on the fiber as such and may therefore be fluxed to encase the fibers as hereinbefore described.

Not only does the method of this invention produce a paper directly on the paper machine as waterproof and water repellent as that dipped in melted paraffin, but this is accomplished with much less wax than is necessary in the dipping process and without the presence of an apparent coating of wax on the surface.

40 Other cellulosic material besides sulphite pulp might, of course, be used, but this is a stock preeminently suited for the manufacture of food containers, particularly when bleached, because of its freedom from substances which might contaminate the food.

In place of forming the entire board or paper with the paraffin therein, it may be formed with two or more plies, one or more 45 plies, which are intended to be in contact with the food being formed of stock containing the paraffin, and the outer ply or plies not having the paraffin therein. This may be done on a multi-cylinder machine, the stock for some of the cylinder molds containing the dispersed waterproofing material and the stock for the other molds having no such material. The waterproofing material being in dispersed condition in the stock in no way hinders the interfelting of the two or more plies, as they are formed and brought together on the multi-cylinder machine, so that a proper felted union of the waterproofed and non-waterproofed plies of the finished product is assured. For example, 50 the inner liner may be made of stock com-

prising 70 to 90 parts of sulphite pulp, 5 to 30 parts of the paraffin dispersion product, and 10 parts of silicate of soda, to which 5 to 25 parts of alum may be added before the stock is run in order to precipitate the 70 paraffin on the pulp. The 10 parts of silicate of soda are merely added to insure sufficient silicate to properly coagulate and bring down the paraffin on the pulp and can be omitted in case the silicate in the dispersion 75 product appears to be sufficient to produce the desired action. The outer liner may be formed of any suitable cellulosic stock, such for example, as 100 parts of sulphite pulp, 5 parts of rosin size, 5 parts of alum. 80

A somewhat cheaper grade of paper or board suitable for oyster pails and the like may be made by the use of cheaper cellulose fiber in the outer ply, such for example, as newspaper pulp. A board particularly suitable, for instance, for milk bottle caps, may have its cellulosic material composed of 50 parts of easily bleached sulphite pulp and 30 parts of ground wood pulp. 85

A sanitary waterproof wrapping paper 90 for food products may be produced from 65 parts of sulphate pulp and 35 parts of paraffin dispersion product.

While various waxes, gums, rosins or resins may be dispersed by subjecting them 95 to treatment similar to that hereinbefore described, paraffin is preferable for food containers or wrappers because of its chemical purity, its ability to stand low temperatures without becoming excessively brittle, 100 its clean appearance, and its compliance with all of the various pure food laws.

A very desirable building paper, or box-board, may be produced by employing the paraffin or other waterproofing dispersion 105 product in the outer plies of the board or paper and in the inner plies using a cheaper waterproofing agent, such as asphalt emulsion, for example, the emulsion known to the trade as K-B emulsion which comprises 110 an emulsion of asphalt with a colloidal clay solution. Thus the furnish for the top and bottom liners may comprise 50 parts of newspaper, 50 parts magazine stock, 20 parts of paraffin dispersion product, and 20 parts of 115 alum, while the middle filler may comprise 100 parts of news, 100 parts of K-B emulsion (dry or 200 parts wet), 15 parts of silicate of soda, 20 parts of alum. Such paper is waterproof throughout and can be 120 run readily on the paper machine. Where asphalt emulsion alone is employed as a waterproofing agent, it is usually necessary to apply top and bottom liners without the emulsion in order to prevent the material 125 from sticking to the blanket and the drying rolls of the machine. As before noted the paraffin dispersion product promotes rather than hinders the proper running of the paper in the machine, since it acts as a lu- 130

briant and prevents sticking to the parts of the machine with which it comes into contact.

A dispersion product suitable for water-proofing paper by the method hereinbefore described but containing a large proportion of carnauba wax may be made by substituting for paraffin and rosin in the example heretofore given, 500 parts of rosin and 500 parts of carnauba wax. It is also possible to form a dispersion of carnauba wax alone in the silicate of soda solution by the hereinbefore described method, though the presence of some rosin or Montan wax causes the dispersion to be somewhat finer. Similarly the amount of paraffin may be decreased and the amount of rosin increased, 500 parts of paraffin and 500 parts of rosin and 50 parts of Montan wax being satisfactory.

I do not herein claim the paper products herein-described, this subject matter having been divided out from this application and being claimed in my application Serial Number 22,394 filed June 1, 1926, nor do I claim herein the aqueous dispersions or the process for making these dispersions, these subjects matter being claimed in my application Serial Number 673,216 hereinbefore mentioned.

Having thus described this invention it should be evident that many modifications and changes might be made therein without departing from its spirit or scope as defined by the appended claims.

I claim:

1. The method which comprises mixing with beater stock a dispersion product of water-proofing material in an aqueous solution of sodium silicate, adding a precipitant, and running off on a paper machine.

2. The method which comprises mixing with beater stock, a dispersion product of paraffin in sodium silicate, adding a precipitant, and running off on a paper machine.

3. The method of producing a waterproof and water repellent paper, which comprises melting a waterproof and water repellent material, adding the melted materials to a hot aqueous solution while it is being thoroughly stirred, suddenly cooling the mixture below the melting point of the material to solidify it in finely dispersed condition, adding the resultant product to fibrous beater stock, precipitating the dispersed material on the fibers, running off on a paper machine, and fluxing the dispersed material.

4. The method of producing a waterproof and water repellent paper, which comprises melting waterproof and water repellent material, adding the melted material to a hot aqueous solution of sodium silicate while agitating the same, and thoroughly mixing, and then suddenly chilling the mixture to

solidify the material in finely dispersed condition, adding the resultant product to fibrous beater stock, adding another precipitant to form a coagulant with the silicate of soda to fix the dispersed material on the fibers, running off on a paper machine and subjecting to a temperature above the melting point of the material until it is fluxed and coalesced about the fibers.

5. The method of producing a waterproof and water repellent paper, which comprises melting paraffin and dispersing agent, adding the melted mass to a hot aqueous solution and thoroughly mixing therewith, rapidly chilling the mixture below the melting point of the paraffin while continuing the agitation to solidify the paraffin and dispersing agent in dispersed condition, adding the product to fibrous beater stock, precipitating the dispersed material on the fibers, sheeting on a paper machine, and subjecting the sheet to a temperature above the melting point of the paraffin and dispersing agent whereby they are fluxed and coalesced throughout the sheet.

6. The method of producing a waterproof and water repellent paper, which comprises melting together paraffin and a wax having a higher penetrability and a lower surface tension than the paraffin, adding the melted mixture to a hot solution of silicate of soda while it is being agitated, then cooling the mixture below the melting point of the paraffin and wax while the agitation is continued to cause the paraffin and wax to become solidified in finely dispersed condition, adding the resultant product to fibrous beater stock, adding a precipitant capable of coagulating with the silicate of soda and fixing the dispersed material on the fibers, sheeting on a paper machine, and subjecting the sheet to a temperature above the melting point of the paraffin and wax to cause them to coalesce throughout the sheet.

7. The method of producing a waterproof and water repellent paper, which comprises melting together paraffin, rosin and Montan wax, pouring the melted mixture into a hot silicate of soda solution while agitating the same, and adding cold water while continuing the agitation to solidify the paraffin, rosin and Montan wax in finely dispersed condition, adding the resultant product to fibrous beater stock, adding a precipitant capable of coagulating with the silicate of soda to fix the dispersed materials on the fibers, sheeting on a paper machine, and subjecting the sheet to a temperature above the melting point of the paraffin, rosin and Montan wax to cause them to coalesce throughout the sheet.

In testimony whereof I have affixed my signature.

ALBERT L. CLAPP.